

## UNITED STATES PATENT OFFICE

2,638,446

LUBRICANT FOR PNEUMATIC TOOLS AND  
THE LIKE

Jones I. Wasson, Union, N. J., assignor to Standard Oil Development Company, a corporation of Delaware

No Drawing. Application May 19, 1950,  
Serial No. 163,079

2 Claims. (Cl. 252—33.4)

1

The present invention relates to a lubricating composition especially adapted for pneumatic tools, such as rock drills, and the like. The invention further pertains to a composition which is adapted for the lubrication of equipment which is operated under adverse conditions of dust, moisture, chemical fumes, and the like, where ordinary lubricants have been found to be somewhat inadequate.

In the lubrication of pneumatic tools, such as rock drills and other equipment operated in mines and under dusty and wet conditions, some difficulty has been encountered in lubrication and care. Rock drills are operated frequently under conditions where the surrounding atmosphere is substantially saturated with moisture vapor and permeated with dust, fumes of sulfur, and other active materials which quickly corrode and cause wear and other deterioration of the equipment.

Aside from problems of corrosion, equipment of the general types mentioned above may be operated under conditions where high unit stresses are applied to its parts. In such cases, it is desirable that a lubricant have greater load-bearing properties, or oiliness, or lubricity, than conventional mineral oil lubricants possess.

The general problem of lubricating rock drills and related equipment has been recognized previously. Some efforts have been made to provide a satisfactory lubricant for the severe uses described above. Thus, in the U. S. patent to Sproule and King, No. 2,479,424, there is described a rust inhibiting lubricant consisting of mineral oil containing as additives small quantities of the partial esters of polyhydric alcohols, for example, sorbitan or pentaerythritol monooleates or monostearates. Various other prior art compositions have employed certain fatty oils, such as rapeseed oil, as modifiers for the conventional mineral base lubricant. Products of this type which are commonly employed as pneumatic drill lubricants have consisted of mineral lubricating oils blended with about 5 to 15% of a thickened fatty oil, such as blown rapeseed oil. In certain respects, these products have shown quite satisfactory lubricating properties. However, they are frequently unsatisfactory in solution stability, i. e., sludging or separation of the modifier frequently occurs, as well as in load-carrying and in rust-preventive properties.

In order to meet the various requirements for lubricants for the pneumatic tools used in severe service, especially underground service, such as rock drills and equipment commonly operating under similar conditions, it appears to be necessary that the several properties of good load-carrying, ability to lubricate in the presence of moisture, resistance to rust, and resistance to other corrosion, be combined compatibly and stably in a single composition. Individual agents for each of these several functions are known in specific

2

environments, but their combination into a stable, sludge-free lubricant having all the desired properties for specialized service is another matter.

According to the present invention, these properties may be combined in a very satisfactory manner by blending with a suitable mineral base lubricating oil, preferably one of viscosity between about 50 and 500 S. S. U. at 100° F., proportions of 0.1 to 4% by weight, based on the total composition, of degras, 0.05 to 5% of a rust inhibiting and water-emulsifying agent, such as an oil-soluble metal sulfonate of alkali or alkaline earth metal, plus about 0.5 to about 10% of a compatible extreme pressure agent in the form of a sulfurized fatty oil, such as sperm oil or other and comparable animal fat, such as lard oil, sulfurized to a sulfur content of 2 to 30% by weight, and about 0.05 to about 3% of a synergistic oiliness agent and rust inhibitor, preferably in the form of an ester of an acid of phosphorus, such as tricresyl phosphate or phosphite, or the corresponding trialkyl esters, such as tributyl phosphate or phosphite. It is also desirable to add a small amount, for example, 0.05 to about 5% maximum of a viscous hydrocarbon polymer. The latter ingredient adds to the tackiness and improves the viscosity index of the lubricant. It increases the resistance of the lubricant to moisture so that it adheres to the part to be lubricated more effectively when water is present. The preferred polymer is a polybutene having a molecular weight of not less than 2,000 and not more than 100,000, preferably between 10,000 and 50,000. Other essentially hydrocarbon polymers and copolymers, such as natural rubber, synthetic rubber like butyl rubber, and polystyrene and alkylated polystyrene may be used, provided they are sufficiently oil-soluble to remain in solution and provided they are compatible with the other ingredients.

Sulfurized degras may be combined with unsulfurized degras, and thus replace the sulfurized sperm oil or other animal fat. In a broad sense, a combination of sulfurized and unsulfurized animal fat or equivalent, seems to be required along with the oiliness and thickener or tackiness additives.

The preferred range of ingredients is from about 86 to about 97% by weight of lubricating oil with 1 to 3% degras, 0.1 to 2% of metal sulfonate, calcium or sodium sulfonate being preferred, particularly the former, about 1 to 5% of sulfurized fatty oil, preferably sperm oil, with sulfur content between 2 and 30%, preferably about 10 to 20%, about 0.5 to 2% of the oiliness agent, tricresyl phosphate being preferred for oiliness although other esters mentioned above are almost as satisfactory, and about the same proportions, namely 0.5 to 2% of a polymer, preferably polybutene or a viscous polymer

of similar properties. A broader range preferred is about 72 to 99% of lubricating oil (preferably, but not necessarily, of mineral base), 0.1 to 5% of degras, 0.05 to 10% of sulfurized fatty material, (or a combination of 0.15 to 15% of sulfurized and unsulfurized fatty material of animal origin) plus the sulfonate, ester, and polymer, as given above.

Table I

| Composition                                                                                                                                                                                       | Load Carrying <sup>1</sup><br>(Almen Test) | Steam Emulsion Number <sup>2</sup> | AN-H-31 Humidity Cabinet, Hrs. <sup>3</sup> |
|---------------------------------------------------------------------------------------------------------------------------------------------------------------------------------------------------|--------------------------------------------|------------------------------------|---------------------------------------------|
| Desired Mineral Oil (without additives)                                                                                                                                                           | Weights 12<br>2                            | 1,200+<br>100                      | 100+<br>1                                   |
| Example I                                                                                                                                                                                         |                                            |                                    |                                             |
| Mineral Oil +<br>3% Sulfurized Sperm Oil<br>1% Tricresyl Phosphate<br>1% Polybutene (15,000-<br>30,000 mol. wt.)<br>2% Degras<br>0.6% Calcium Sulfonate<br>Mineral Oil + 7% Blown<br>Rapeseed Oil | 13                                         | 1,200+                             | 600                                         |
|                                                                                                                                                                                                   | 5                                          | 1,200+                             | 24                                          |

<sup>1</sup> Journal of Institute of Petroleum, vol. 32, 1946.

<sup>2</sup> ASTM D-157-36.

<sup>3</sup> U. S. Army-Navy Specification.

The combination of additives shown in Example I above appears to be necessary to obtain all of the desirable properties. Tests made on blends in which one or more of the additives were left out resulted in unsatisfactory products from the standpoint of meeting all requirements. This was particularly true in the case of meeting the critical load-carrying and humidity cabinet tests. For example, blends similar to Example I, except not containing sulfurized sperm oil, carried only 2 to 3 weights in the Almen test and showed humidity cabinet lives of only 72 hours. Other blends containing all of the additives except tricresyl phosphate carried only 2 to 3 weights in the Almen test and gave only 72 hours humidity cabinet lives. Similar results were obtained on blends without both the sulfurized sperm oil and tricresyl phosphate. Results obtained on these blends are presented in Table II.

Table II

| Composition                                                                                      | Load Carrying<br>(Almen Test) | AN-H-31<br>Humidity Cabinet<br>(Hrs.) |
|--------------------------------------------------------------------------------------------------|-------------------------------|---------------------------------------|
| Example II                                                                                       |                               |                                       |
| Mineral Oil +<br>1% Tricresyl Phosphate<br>1% Polybutene<br>2% Degras<br>0.6% Calcium Sulfonate  | 2-3                           | 72                                    |
| Example III                                                                                      |                               |                                       |
| Mineral Oil +<br>3% Sulfurized Sperm Oil<br>1% Polybutene<br>2% Degras<br>0.6% Calcium Sulfonate | 2-3                           | 72                                    |
| Example IV                                                                                       |                               |                                       |
| Mineral Oil +<br>1% Polybutene<br>2% Degras<br>0.6% Calcium Sulfonate                            | 2-3                           | 72                                    |

The above data show the marked inferiority of the experimental materials as compared with the product of Example I (Table I). The mineral oil used in Examples I to IV was the same type and grade in each instance. The presence of polybutene appears to be necessary to give the blends adhesive properties, which prevent the oil from being displaced or thrown off the equipment during service.

10 While mineral oil is the preferred base lubricant, it is possible also to use synthetic ester lubricants, such as the dibasic acid esters and the glycol and glycol-ether type lubricants, which have recently come into use. Mineral oil products are generally less expensive and are usually preferred although specific applications may call for the ester type or glycol type oils.

The humidity cabinet test given above is the standard humidity cabinet rusting test wherein 20 a polished steel strip is coated with the lubricant and kept under conditions of approximately 100% relative humidity at a temperature of 120° F. until first rusting appears. As indicated in the tables above, it is desired to have a humidity cabinet life of at least 100 hours. Plain mineral oil rusts in about one hour. The composition of the present invention (Example I) ran 600 hours before rusting, whereas a conventional prior art rock drill lubricant containing 7% blown rapeseed oil gave a humidity cabinet life of only 24 hours. The products of Examples II, III and IV were of intermediate quality.

What is claimed is:

- 35 1. A lubricant for pneumatic tools, and the like, consisting essentially of about 86 to 97 parts by weight of mineral base lubricating oil having a viscosity between 50 and 500 S. S. U. at 100° F., 1 to 3 parts of degras, 0.1 to 2 parts 40 of oil-soluble calcium petroleum sulfonate, 1 to 5 parts of sulfurized sperm oil containing 10 to 20% of sulfur, 0.5 to 2 parts of tricresyl phosphate and 0.5 to 2 parts of polybutene of molecular weight between 10,000 and 50,000.
- 45 2. A composition having approximately the following formula in percentages by weight:
- 92.4% mineral lubricating oil  
2.0% degras  
0.6% oil-soluble calcium sulfonate  
50 3.0% sulfurized sperm oil (10 to 20% by weight of sulfur)  
1.0% tricresyl phosphate  
1.0% polybutene of molecular weight between 15,000 and 30,000.

55 JONES I. WASSON.

References Cited in the file of this patent

UNITED STATES PATENTS

- 60 Number Name Date  
2,184,952 Zimmer Dec. 26, 1939  
2,270,577 Bergstrom Jan. 20, 1942  
2,398,429 Hughes Apr. 16, 1946  
65 2,453,833 Davis Nov. 16, 1948